

# UNITED STATES PATENT OFFICE.

GADIENT ENGI, OF BASEL, SWITZERLAND, ASSIGNOR TO SOCIETY OF CHEMICAL INDUSTRY IN BASLE, OF BASEL, SWITZERLAND.

## PROCESS FOR DYEING AND PRINTING WITH DERIVATIVES OF NAPHTHAZARIN.

1,202,821.

Specification of Letters Patent.

Patented Oct. 31, 1916.

No Drawing.

Application filed June 18, 1913. Serial No. 774,363.

To all whom it may concern:

Be it known that I, GADIENT ENGI, doctor of philosophy and chemist, a citizen of the Swiss Republic, and resident of Basel, Switzerland, have invented a new and useful Process for Dyeing and Printing with Derivatives of Naphthazarin, of which the following is a full, clear, and exact specification.

10 It is known that naphthazarin and some of its derivatives, as for instance arylnaphthazarins, are only capable of employment for dyeing wool and printing wool and cotton either in the form of bisulfite compounds 15 or in the form of sulfonic acids. For the dyeing of cotton these products have not, heretofore, been capable of employment. I have now found that a series of condensation and transformation products of 20 naphthazarin and of its homologues and substitution products yield by their treatment with reducing agents leuco compounds soluble in alkalis, having the surprising property of an affinity for textile fibers rendering them well suited for dyeing and printing the same by the methods known for the vat-dyestuffs, whereby gray, brown, 25 brown-black, green-black, blue-black to deep-black dyeings and printings are obtained, having an excellent fastness particularly when subjected to a subsequent treatment with metal salts.

I have ascertained that the property of dyeing textile fibers from an alkaline vat is 30 a specific characteristic of nearly all condensation and transformation products of naphthazarin, this latter being itself remarkably devoid of the said property. Thus the following groups of compounds of the naphthazarin series are, for instance, suitable for 35 vat-dyeing.

(a) the arylamino derivates obtainable by the condensation of naphthazarin and of its substitution products with aromatic amines 40 and their sulfonic or carboxylic acids.

(b) the transformation products obtainable by heating naphthazarin, its substitution products of the arylamino derivates specified under paragraph (a) in diluents or 45 solvents with or without addition of alkalis, alkali metal sulfids, alkaline earth, metal sulfids or other salts.

(c) the condensation products obtainable by the action of bodies containing the group



55 as for instance indoxyl, oxythionaphthene, phenols, naphthols, anthranol, etc., on naphthazarin, its substitution products or their leuco-derivatives, or the so called intermediate products of naphthazarin, or the compounds specified in the foregoing paragraphs (a) and (b).

(d) the condensation products obtainable 60 by the action of organic compounds containing one or several primary, secondary or tertiary amino groups on naphthazarin, its substitution products or the bodies specified in the foregoing paragraphs (a) to (c).

70 The vegetable fibers dyed according to the present process have the property coloring cold sulfuric acid of 66° Bé. gray-blue and hot soda-lye of 7.5 per cent. slightly green, when they are laid in the said solvents, but 75 do not color cold soda-lye of 2.5 per cent. and color only by traces hot hydrochloric acid.

The employment of the specified products 80 as vat-dyestuffs for dyeing and printing will be illustrated by the following examples:

### Example 1.

3 to 4 parts of the condensation product of 85 naphthazarin and anilin obtained according to Example 2 of the German Patent No. 101,525, are transformed to a paste with 3 to 4 parts of soda lye of 30 per cent. To this paste are added 300 parts of hot water and 2 to 3 parts of sodium hydrosulfite (powder) 90 and the mixture is heated for a short time, whereby a brown-orange solution is produced. By adding hot water this solution is diluted to the desired volume and the fibers are dyed in the same at a temperature of 60 95 to 90° C., while common salt (30 to 40 grams per lit.) is added for about half an hour, squeezed out, exposed to the air for about 30 minutes and finally rinsed. When 50 to 60 parts of cotton are employed for the above 100 specified quantity of dye-stuff, there are obtained black dyeings which become more fast by a subsequent treatment with metal salts.

In an analogous manner the other con-

dersation products soluble in alkalis resulting from the action of other aromatic amines on naphthazarin according to the German Patent No. 101,525 can be employed for dyeing purposes.

*Example II.*

3 parts of an arylated product insoluble in alkalis, obtained by boiling for several hours naphthazarin with alcohol in presence of an aromatic amine, are transformed to a vat according to the indications of Example I. The resulting vat is added to the dyeing bath to which 80 grains of common salt have been added per liter and the cotton is then introduced in the bath. The said cotton is dyed for  $\frac{1}{2}$  hour at 80° C., squeezed out, oxidized during  $\frac{1}{2}$  hour by exposure to the air, rinsed and the dyeings are finally treated, for  $\frac{1}{2}$  hour at 90° C., with a bath containing 5 grams of copper sulfate or 5 grams of potassium chromate per liter. The dyed cotton is afterward rinsed and dried.

25 When the employed condensation product insoluble in alkalis is derived from anilin, a deep black is obtained, which has an excellent fastness to washing, light, acids and a satisfactory fastness to chlorin. By printing oxidizing discharges on goods thus dyed, pure whites are obtained.

The corresponding condensation product derived from paraphenylenediamin gives a more reddish black having besides the same fastness to washing, light and hot acids a greater fastness to chlorin. The condensation product of naphthazarin with benzidin furnishes a more bluish-black, while the product derived from naphthazarin and orthophenylenediamin gives black-brown vat-dyeings. The corresponding products derived from naphthazarin and the homologues of anilin, monoethylanilin, dimethyl-anilin, naphthylamin, diphenylamin, mono-aminodiphenylamin, diamino-diphenylamin, aminoanthraquinone, etc., give also black dyeings of more greenish, more bluish or more reddish tints than the dyeings obtained with the condensation product derived from anilin. Also the condensation products obtained by the condensation of naphthazarin with sulfonic or carboxylic acids of aromatic amines, for instance by boiling in an alcoholic solution or suspension, give black vat-dyeings. Thus a fast black is for instance obtained with the condensation product of naphthazarin with sulfanilic acid, the tints of the dyeings being somewhat more greenish than those obtained with the product derived from anilin. The corresponding condensation products prepared with 1:8-naphthylaminosulfonic acid, or 2:6-naphthylaminomonosulfonic acid, or anthranilic acid yield some-

what more reddish black tints, while the condensation products derived from amido-salicylic acid dyes more bluish-black.

*Example III.*

If instead of the arylated naphthazarins specified in the foregoing examples, the transformation product, obtained by a long boiling of naphthazarin with water, is employed, black dyeings of good fastness to washing and to light are also obtained.

Analogous dyeings are obtained by the employment of the transformation products resulting from the boiling of naphthazarin with water and alcohol or another solvent or diluent, to which alkalis, as for instance soda lye, soda or ammonia, alkali sulfids, as for instance potassium sulfid, or other salts, as for instance sodium acetate, sodium phosphate, etc., have been added.

*Example IV.*

4 parts of the condensation product resulting from the condensation of naphthazarin with oxythionaphthene are transformed with soda lye and hydrosulfite to a vat showing a red-orange coloration. The cotton yarn is introduced in this vat and dyed therein for half an hour at 80° C., squeezed out, exposed to the oxidizing action of air, rinsed and eventually treated finally with a hot soap solution. A beautiful deep-black is thus obtained. On wool black-gray tints are obtained.

*Example V.*

4 parts of the condensation product obtained by boiling naphthazarin with water or an aqueous solution of sodium sulfid and by treating the resulting transformation product subsequently with anilin or para-phenylenediamin are transformed into a vat, which is employed to dye cotton in the above specified manner. The dyeing thus obtained after exposure to the air is treated with a hot bath containing copper sulfate or potassium chromate. The deep-black tints so obtained are of excellent fastness.

Analogous dyeings are obtained with the condensation products obtained by boiling naphthazarin with water and soda or sodium acetate and by subsequent treatment with aromatic mono- or polyamines.

For the employment of the specified derivatives of naphthazarin to printing purposes, I proceed as follows:

*Example VI.*

60 to 80 grams of dyestuff, 100 grams of soda lye of 36° Be, 60 grams of glycerin, 300 grams of water, 80 grams of hydrosulfite (powder), 360 grams of alkaline thickening are heated together to 80° C.; after cooling to 50-60° C., 80 gr. hydrosulfite

N. F conc. are added. This printing color is printed on the fabric as usual or, if desired, the fabric may be prepared with glucose, and the fabric is then dried and steamed for 5 minutes in the Mather-Platt, at about 102° C. The goods are then passed through a bath containing 5 grams potassium chromate or copper sulfate, rinsed and dried. The prints thus obtained are of deep black tints 10 and show the same fastness as the vat dyes.

*Example VII.*

80-100 grams of dyestuff  
 15 400 grams of alkaline thickening  
 100 grams of glycerin  
 100 grams of glucose and  
 250 grams of water are heated to 70° C. and then  
 20 50 grams of hydrosulfite N. F conc. are added at 50° C.  
 1 kg.

After printing, the goods are steamed for 25 5 minutes in the Mather-Platt at 100-102° C., and thereafter treated with a bath containing 5 grams of potassium chromate per liter, rinsed and soaped with boiling soapy water.

*Example VIII.*

A printing color consisting of 250 grams of dyestuff (paste), 650 grams of alkaline thickening, and 100 grams of glycerin is printed on a fabric prepared with glucose. 35 The fabric is then dried, steamed in moist steam free of air in the Mather-Platt for 3 minutes, subjected to oxidation and sub-

sequent treatment with potassium chromate or copper sulfate.

In an analogous manner all compounds 40 of the naphthazarin series above specified may be employed for dyeing and printing.

What I claim is:

1. The described process of producing gray to black shades on textile fibers consisting in treating naphthazarin derivatives with alkaline reducing agents, applying the leuco compound thus produced on the fibers and finally oxidizing the same on the fibers. 45

2. The described process of producing gray to black shades on the textile fibers consisting in treating naphthazarin derivatives with alkaline reducing agents, applying the leuco-compound thus produced on the fibers, 55 oxidizing the same on the fibers and finally treating the dyed material with hot solutions of metal salts operable to impart fastness to the shade produced.

3. As a new article of manufacture, a textile fiber dyed with the oxidation products of a leuco compound of naphthazarin-derivatives, the dyed fiber coloring cold sulfuric acid of 66° Bé. gray-blue, hot hydrochloric acid of 21° Bé. only by traces and hot soda 65 lye of 7.5 per cent. slightly green, but not coloring cold soda lye of 7.5 per cent.

In witness whereof I have hereunto signed my name this 4th day of June, 1913, in the presence of two subscribing witnesses.

GADIENT ENGI.

Witnesses:

GEO. GIFFORD,  
 AMAND RITTER.